

## UNITED STATES PATENT OFFICE

2,221,248

## MAGNESIUM BASE ALLOY

Joseph D. Hanawalt and John C. McDonald, Midland, Mich., assignors to The Dow Chemical Company, Midland, Mich., a corporation of Michigan

No Drawing. Application November 13, 1939,  
Serial No. 304,125

## 3 Claims. (Cl. 75—168)

The invention relates to magnesium base alloys. It more particularly concerns alloys of this nature having a high degree of formability coupled with other improved physical properties, such as increased tensile and yield strengths.

Magnesium alloys are enjoying increasing use in the structural and mechanical arts where a light weight metal is highly desirable, such as for use in making large castings, forgings, and the like. However, the use of these alloys in the rolled form to make sheet metal articles requiring forming operations, such as bending, drawing, and the like, has not progressed as rapidly due to the fact that in general alloys of good formability permitting relatively sharp bends to be made without the article developing external cracks usually have inferior characteristics as regards their tensile and yield strengths.

It is, accordingly, the principal object of the invention to provide a magnesium base alloy which may be made into rolled sheet or the like, possessing a sufficient degree of ductility or formability to be sharply bent, drawn or otherwise shaped while having improved tensile and yield strengths.

Other objects and advantages will be apparent as the description of the invention proceeds.

Our invention resides in the discovery that a magnesium base alloy composed of 0.3 to 8 per cent of silver, 0.05 to 1 per cent of calcium, 0.1 to 3 per cent of manganese, 0.1 to 8 per cent of zinc, and from 0.1 to 8 per cent of tin, the bal-

to 6 per cent of silver, 0.1 to 0.3 per cent of calcium, 1 to 3 per cent of manganese, 2 to 5 per cent of zinc, and from 4 to 7 per cent of tin. Alloys containing the higher percentages of alloying ingredients, while still having good ductility have exceptionally high yield and tensile properties and thus are also suitable for use in casting operations.

The specific proportions of each alloying metal and the total amount of the added metals to be employed in these new alloys depends on the use for which the alloy is intended. In general it is preferable to use alloys containing more than about 82 per cent magnesium and less than 18 per cent of the total added metals. For example, in alloys wherein high ductility or formability is of prime importance, the total added alloying metals should not materially exceed 10 per cent; while in those instances where high yield and tensile strengths are desirable in both the cold rolled and annealed state, the percentage of total added metals should preferably be above 12 per cent.

The following table, which lists some of the properties of rolled sheet metal made from our new alloy and compares these properties with those of a related alloy, illustrates the improvement in yield strength, tensile strength, and ductility or formability, as represented by the per cent increase in elongation of the new alloy over the corresponding properties of closely related alloy.

Table

| 35 | Nominal composition in percent<br>(magnesium=remainder) |     |     |     |       | Annealed                          |                                     |                                   | Cold rolled                       |                                     |                                   | 35 |
|----|---------------------------------------------------------|-----|-----|-----|-------|-----------------------------------|-------------------------------------|-----------------------------------|-----------------------------------|-------------------------------------|-----------------------------------|----|
|    | Ag.                                                     | Ca. | Mn. | Sn. | Zn.   | Yield strength<br>in lbs./sq. in. | Tensile strength<br>in lbs./sq. in. | Percent elongation<br>in 2 inches | Yield strength<br>in lbs./sq. in. | Tensile strength<br>in lbs./sq. in. | Percent elongation<br>in 2 inches |    |
| 40 | 1.2                                                     | 0.3 | 0.3 | 5.1 | ----- | 22,000                            | 35,000                              | 7                                 | 31,000                            | 38,000                              | 2                                 | 40 |
|    | 1.2                                                     | 0.3 | 1.0 | 5.3 | 1.8   | 25,000                            | 39,000                              | 12                                | 33,000                            | 43,000                              | 8                                 |    |
|    | 1.1                                                     | 0.2 | 1.1 | 5.1 | 3.3   | 23,000                            | 39,000                              | 15                                | 40,000                            | 46,000                              | 3                                 | 45 |

45 ance being substantially all magnesium, is endowed with the afore-mentioned properties. While the properties of improved formability or ductility coupled with increased tensile and yield 50 strengths are manifest over the entire range of composition indicated, we have found that in general the preferred combination of properties, such as the most desirable, ductility for forming operations coupled with high tensile and yield 55 strengths is found in alloys containing from 1

The properties listed in the above table under the section headed by the term "annealed" were obtained by first rolling the alloys at a temperature between about 500° to 700° F., and thereafter annealing them at various temperatures through a temperature range of from 400° to 800° F. The properties selected for the table were those of the annealed specimens which exhibited the maximum elongation. The properties listed under the section headed "cold rolled" 55

were obtained by subjecting specimens of the alloys which had been hot rolled at a temperature of from 500° to 700° F. to additional rolling in the cold state to bring about a total reduction in thickness of from 2 to 10 per cent. The properties selected for the table were those of the cold rolled specimens which showed the greatest tensile and yield strengths, while having at least a 1 per cent elongation in 2 inches.

5 10 By a comparison of the properties listed in the above table, it will be observed that the combined properties of our new polynary alloys are superior to those of the parent quintary alloys having similar percentages of alloying ingre-

15 20 25 30 dents. For example, it will be noted that the per cent elongation is greatly improved while the yield and tensile strength in both the annealed and cold rolled state also show marked improvement. Similarly alloy compositions containing other percentages of the alloying ingredients show improved properties over those of the related alloys.

While the new alloy is most useful in wrought form, such as sheets, due to its formability characteristics, it may also be suitably used in making castings, forgings, extruded forms, and the like. It is further pointed out that our new alloy is amenable to solution and precipitation heat treatments, which, accordingly, modify its properties.

The new alloy may be compounded in any

ways known to the art, such as by adding the alloying ingredients to the molten magnesium under a suitable flux. The flux should be substantially free from magnesium chloride, if the calcium content of the alloy is to be above 0.3 per cent. In those instances where an alloy is to be compounded containing less than 0.3 per cent of calcium, magnesium chloride may be present in the flux without exerting a deleterious effect, but in this case it is usually desirable to add the calcium last and without too much stirring in order that the loss of calcium into the flux will be substantially prevented.

5 10 15 20 25 30

We claim:

1. A magnesium base alloy containing from 0.3 to 8 per cent of silver, 0.05 to 1 per cent of calcium, 0.1 to 3 per cent of manganese, 0.1 to 8 per cent of zinc, and from 0.1 to 8 per cent of tin, the balance being magnesium.

2. A magnesium base alloy containing from 1 to 6 per cent of silver, from 0.1 to 0.3 per cent of calcium, 1 to 3 per cent of manganese, 2 to 5 per cent of zinc, and from 4 to 7 per cent of tin, the balance being magnesium.

3. A magnesium base alloy containing from 6 to 8 per cent of silver, 0.3 to 0.7 per cent of calcium, 1 to 3 per cent of manganese, 6 to 8 per cent of zinc, and from 7 to 8 per cent of tin, the balance being magnesium.

JOSEPH D. HANAWALT. 30  
JOHN C. McDONALD.